

Sept. 22, 1936.

E. ROSTAS

2,055,181

PHOTOELECTRIC TUBE

Filed Nov. 26, 1930

FIG. 1



FIG. 2



INVENTOR  
E. ROSTAS

BY

Stanley B. Kent.  
ATTORNEY

## UNITED STATES PATENT OFFICE

2,055,181

## PHOTOELECTRIC TUBE

Ernest Rostás, Paris, France, assignor to Western Electric Company, Incorporated, New York, N. Y., a corporation of New York

Application November 26, 1930, Serial No. 498,290  
In France January 6, 1930

9 Claims. (Cl. 250—27.5)

This invention relates to the manufacture of photoelectric tubes and more particularly to method for producing a light sensitive surface for such tubes.

5 An object of the invention is to effect improvement in the method of supplying photoelectric tubes with an interior coating of photoelectrically active material.

10 A further object of the invention is to effect improvement in the method of activating the photoelectrically active material. Alkali metals such as sodium and potassium are the metals usually employed because these are found to be extremely sensitive to light, but other alkali 15 metals, such as lithium and caesium, sometimes are employed.

20 Various methods are in common use for introducing alkali metals in a pure state into the interior of the glass or like envelope on the inner surface of which the metal is to be deposited as a film to form the cathode.

25 One such method of introducing potassium is that of repeated distillation of the potassium in vacuum. Such a method involves the use of expensive apparatus, consequently tubes produced by this method are quite costly.

30 A feature of the present invention is concerned with an improved method for impregnating the inner surface of the wall of a glass envelope with ions of an alkali metal, such as potassium, by effecting electrolysis between a quantity of molten alkali metal salt contained in the envelope and a quantity of the same salt forming an external bath in which the envelope is partially immersed.

35 In an example of practice of the invention a quantity of molten potassium nitrite is introduced into a glass bulb which is partially immersed in a bath of the same molten salt. Contact is made to each lot of the molten alkali metal salt and an 40 electric current from a suitable source is passed therebetween and through the glass so that electrolysis takes place in the ordinary way and in such a direction that metallic ions from the salt inside the bulb pass into the glass. By this means 45 the sodium or like ions contained in the glass close to the interior surface are replaced by the potassium ions from the molten salt inside the bulb. The bulb is then washed and cleaned thoroughly.

50 An internal filament is now introduced, in the turns of which is placed a small piece of magnesium. The bulb is again highly evacuated and the filament heated to the vaporization temperature of the magnesium which is liberated in the 55 form of a vapor and deposits on the cool portion

of the bulb. Reverse electrolysis is then started by applying a suitable potential between the heated filament and an external bath of molten salt with the result that the potassium ions passed by the first electrolysis into the glass wall from the 5 molten alkali salt, are liberated into the bulb and deposited on the magnesium. This potassium metal is condensed in the form of a light-sensitive layer on the walls of the tube everywhere except on the small area whose outside surface is exposed to the molten potassium salt. This clear portion of the tube wall serves as a window for admission of light during the operation of the tube. A small shield prevents deposition of the magnesium and potassium metals in such a place 10 as to cause electrical leakage.

20 One method for activating the light sensitive layer formed as described above, is effected by introducing a very low pressure of hydrogen of the order of .001 millimeter of mercury and lighting the filament previously introduced into the bulb, in the presence of this gas. Hydrides of the metal comprising the sensitive layer are formed and the activation is completed without any glow discharge.

25 For a more complete understanding of the method and apparatus involved in this invention attention is called to the accompanying drawing and following description.

30 Fig. 1 is a front cross-sectional view of apparatus for effecting impregnation of the inner walls of a tube container with an alkali metal by electrolysis.

35 Fig. 2 is a front cross-sectional view of apparatus for effecting release of such metal by reverse electrolysis.

40 According to one feature of the present invention a glass bulb into which it is desired to introduce an alkali metal is placed in a bath of molten alkali metal salt there being also some molten alkali metal salt of the same character inside the bulb. Contact is made to each lot of molten alkali metal salt and an electric current is passed therebetween and through the glass so that electrolysis takes place in the ordinary way and in such a 45 direction that metallic ions from the salt inside the bulb pass into the glass. By this means, the sodium or like contained in the glass close to the interior surface is replaced by the metallic ions from the molten salt inside the bulb. The bulb is 50 then washed, cleaned and exhausted by pumping, an internal filament being introduced. Reverse electrolysis is then started with the result that the metallic ions of the alkali metal, passed by the first electrolysis into the glass from the molten 55

alkali salt, are liberated into the bulb thus producing alkali metal in an evacuated bulb.

Referring now to Fig. 1 a metal container 1 is supported by any suitable type of supporting stand, not shown. A glass container 5 having an electrode 14 from which a conductor 13 passes to the exterior is partially immersed in a mass of molten potassium nitrite 4 there being also another mass of the molten potassium nitrite 10 6 of the same character, within the container 5. The heat necessary to keep the potassium nitrite in a molten state is supplied from a Bunsen burner 7 supported in any suitable manner. The glass container 5 has an exhaust tube 16, a hydrogen inlet tube 24 and a metal rod 9 which makes contact with the molten salt 6 on one end while the other end is connected by a wire to the positive terminal of a battery 10, the negative terminal of the battery being connected through switch 20 11 to the metal container 1 by the binding post 12.

Fig. 2 shows apparatus used for producing reverse electrolysis, in accordance with this invention, and is the same as Fig. 1 with a few exceptions. The same reference numerals have been used in the two figures to indicate identical parts. In this figure the contact rod 9 of Fig. 1 has been replaced by a filament 17, and a shield 19, whose purpose will be described later, is attached to the filament leads at the base of the neck of the glass vessel 5. A battery 20 and a variable resistance 21 are connected in series with the filament 17. An additional battery 22 is included in a circuit between the filament 17 and the exterior molten potassium nitrite 4, contact 35 with the latter being made through the metal container 1, by binding post 12.

According to a preferred example of the process a glass envelope 5 is partially immersed in a bath of molten potassium nitrite 4 and a quantity of molten potassium nitrite 6 is introduced inside the envelope 5 and by an electrolysis method potassium is caused to pass into the glass on the interior surface of the envelope 5. An internal filament 17 is now introduced in the turns of which is twisted a small strip of magnesium 18. The envelope is highly evacuated through tube 16 and is placed in a bath of molten potassium nitrite 4; the filament 17 is then heated and the magnesium 18 is deposited on the cool portion 50 of the wall of the bulb 5, a small shield 19 is used to prevent the magnesium depositing in such position as to cause an electrical leak. A potential from battery 22 is then applied between the filament 17 and the molten nitrite 4 outside the envelope 5 by closing switch 23 and potassium contained in the glass is deposited on the magnesium. If this reverse electrolysis is not carried on too long, only potassium is introduced into the envelope 5, but if the action is carried on longer, sodium in the glass also begins to appear and an alloy of potassium and sodium can be produced in the envelope.

The potassium tubes thus made can be activated with hydrogen in a manner hereinafter described and filled with a gas such as argon. The magnesium coating onto which the potassium is deposited may be produced by evaporating the magnesium supported by the filament in an atmosphere of hydrogen at a pressure of ten millimeters or ten centimeters whereupon the envelope is exhausted and the potassium deposited as described. By this method no suitable shadow of an object in the vessel, so as to form a window, can be obtained, but since the vessel is dipping in the hot nitrite the temperature at that

point is sufficient to remove any magnesium deposited there and thus a good window is obtained on the hot part of the bulb.

According to a modification the envelope 5 is pumped down to a high vacuum by means of a suitable pump connected to the exhaust tube 16 and evaporation of the magnesium 18 and the electrolysis of the photoelectric material are carried out at the same moment instead of consecutively.

It is necessary to activate such tubes and the usual method is to pass a glow discharge through the tube when containing hydrogen at a pressure of  $\frac{1}{10}$  of a millimeter this process being the well known one due Elster and Geitel.

A difficulty with such a process is that the hydrogen eats away the active surface at the point of contact with the lead, so that contact with the sensitive surface is lost.

A method of activating such tubes whereby this disadvantage is avoided is as follows: Hydrogen is admitted at a very low pressure, e. g.,  $\frac{1}{100}$  millimeter and the filament is caused to light. Activation then proceeds without any glow discharge. Although activation by this method will proceed without any discharge, it is sometimes desirable to employ a potential difference of 100 volts between sensitive surface and the filament, the filament being anode. This assists the activation. It is thought that the activation occurs under these conditions on account of the formation of atomic-hydrogen which hydrides the surface more easily than molecular hydrogen. Although this theory is given it is to be understood that the invention is not to be limited thereby. Surfaces produced in this way are five or six times more sensitive after activation than before.

One example of a specific activation in accordance with the foregoing process is as follows: Hydrogen is admitted to the evacuated vessel 5, formed with a sensitive surface of sodium or potassium, through a palladium valve connected to the side tube 24 until the pressure is of the order of  $\frac{1}{100}$  of a millimeter. (See Fig. 2.) The filament 17 contained in the vessel 5 is of tungsten and is heated to a temperature of about 2500° K. Immediately activation begins and the process is then continued until maximum sensitivity is reached. After this the activity falls very slowly. If too much hydrogen is put in, say from .01 to .05 millimeter the activity rises but immediately falls off, but on pumping out the hydrogen through the exhaust tube 16 with the filament 17 alight the activity rises rapidly. It is possible to activate the tube with the filament alight in this way with a voltage applied between the cathode 14 and filament 17 under such conditions that the pressure is insufficient to cause a glow discharge. However, it is preferable not to apply a potential.

While the invention relates primarily to the manufacture of photoelectric tubes, applicant's novel method, as defined in certain of the claims, may obviously find other uses. The various aspects of the invention are defined in the appended claims.

What is claimed is:

1. The method of introducing light sensitive material into a photoelectric tube which comprises impregnating the inside of said photoelectric tube container with a light sensitive material by electrolysis, and subsequently liberating said material by reverse electrolysis.
2. The process of manufacturing a photoelec-

tric cathode which comprises immersing a glass bulb containing molten alkali metal salt in a bath of similar molten alkali metal salt, effecting substitution of the metal ions in the glass bulb with metal ions of the enclosed salt by electrolysis, and liberating in said glass bulb such metal ions to form therein a light sensitive cathode by reverse electrolysis.

3. In the manufacture of a photoelectric tube 10 the process comprising impregnating the inner surface of the tube with metal ions of alkali metal salt by electrolysis, evacuating the tube to a high vacuum, vaporizing magnesium from a heated filament on to the walls of the tube, applying a 15 potential between said filament and an external bath of molten alkali metal salt to effect thereby reverse electrolysis whereby a layer of potassium is deposited on the magnesium.

4. In the manufacture of a photoelectric tube 20 the process comprising impregnating the inner surface of a glass envelope with alkali metal ions by means of electrolysis, depositing magnesium by evaporation of the metal from an internal heated filament on to the walls of the envelope, 25 depositing alkali metal on the magnesium by reverse electrolysis, and activating the magnesium and alkali sensitive surface by lighting said filament in the presence of a very low pressure of hydrogen of the order of .001 millimeter.

30 5. The method of preparing an electrode for a photoelectric device which consists in introducing an alkali metal into a container by electrolysis, vaporizing a metal in said container so that the metal forms a conductive coating upon the inner 35 walls of the container, and then depositing said alkali metal upon said conductive coating by reverse electrolysis.

6. The process of manufacture of a photoelec-

tric tube which comprises introducing molten alkali metal salt into a glass envelope, partially immersing said envelope in a bath of molten alkali metal salt, effecting electrolysis between the two lots of salt to cause metal ions of the salt within the envelope to enter the glass, cleaning and evacuating said envelope, vaporizing a metal to form a conductive coating upon the inner walls of said envelope, depositing alkali metal on said conductive coating by reverse electrolysis, and activating said alkali metal to produce a light sensitive surface.

7. The method of activating without glow discharge a light sensitive surface in a photoelectric tube having a cathode and a filamentary anode 15 comprising evacuating the tube to a high vacuum, admitting to the tube a low pressure of hydrogen, and heating the filamentary anode.

8. The method of introducing light sensitive material into a photoelectric tube which comprises impregnating the inside of said photoelectric tube container with metallic potassium ions obtained by an electrolysis of molten potassium nitrite within the container, and subsequently liberating said potassium ions by a reverse electrolysis between an internal filament and an external mass of molten potassium nitrite.

9. The method of preparing an electrode for a photoelectric tube which consists in impregnating the inner surface of the tube container with metal 30 potassium ions by electrolysis, vaporizing magnesium metal from a heated filament onto the inner surface of the tube container, and by reverse electrolysis causing the said potassium ions to deposit on the interior surface of the said 35 magnesium metal.

ERNEST ROSTÁS.